

## UNITED STATES PATENT OFFICE.

RENÉ COURTIEN, OF MARCUY LEZ COMPIEGNE, FRANCE.

## METHOD FOR PROTECTING FLUID CONTAINERS.

No Drawing. Application filed June 7, 1927, Serial No. 197,844, and in France June 11, 1926.

The present invention relates to methods for protecting fluid containers and has more particular reference to methods for protecting petroleum or gasoline tanks or containers 5 such as the ones used on board aeroplanes, air-ships or like aircraft machines against impacts of all kinds, also against perforations caused by bullets or other missiles or objects and against their disastrous consequences 10 such as the destruction of the aircraft by fire.

A primary object of the invention is to provide a method whereby the tank or container is externally coated with a layer of a resilient, elastic and non-inflammable composition which once set on the said container 15 protects it against impacts and automatically closes up or seals any perforation produced therethrough as by a machine-gun bullet.

A further object of the invention is to provide a method whereby the tank or container is externally coated with a layer of a resilient, elastic and non-inflammable composition which once set on the said container protects it against impacts and automatically seals 25 any perforation produced therethrough as by a machine-gun bullet whilst being also impervious and non-soluble in water so that the efficaciousness of said layer is preserved if the aircraft passes through a moist ambient 30 space or accidentally falls in a mass of water, as in the case of hydroplanes.

Other objects of the invention will readily appear from the following specification and appended claims.

According to the invention, the tank or container is essentially coated with a layer of a composition somewhat similar to the one used for covering printing rollers and made of suitable proportions of ingredients 35 comprising glycerine, a gelatinous substance (such as fish glue, pure gelatine, arabic gum, vegetable glue, gum-lac or the like), a binding substance adapted to harden when it sets (such as glucose, molasses or treacle) and 40 water, the following exemplifying proportions by volume being suitable:

|                           | Parts.   |
|---------------------------|----------|
| Glycerine-----            | 30 to 50 |
| Gelatinous substance----- | 40 to 60 |
| Binding substance-----    | 1 to 2   |
| Water-----                | 10 to 15 |

Experimental tests conducted have disclosed that excellent results can be obtained with a coating of a composition formed

by the admixture of the following ingredients:

|                                     | Parts. |
|-------------------------------------|--------|
| Glycerine-----                      | 39½    |
| Gelatine or fish glue-----          | 48     |
| Commercial glucose or molasses----- | 1½     |
| Water-----                          | 11     |

Similar proportions can also be used with substantially the same results.

The thickness of the coating on the container naturally depends on its size and on the breaking or perforating stresses to which it will be submitted as evidently if the container has to withstand powerful impacts and is exposed to a risk of perforation by big bullets, the coating must be thicker. However in ordinary cases a suitable thickness varies from  $\frac{1}{4}$  to  $\frac{7}{8}$  of an inch.

A convenient way of applying the aforesaid coating consists in first applying a thin layer of an adhesive paint on the outer wall 65 of the container, adhesive paint being that which is commonly used in the art for causing the composition of which printing rollers are usually made to adhere to the supporting axle or mandrel. Such adhesive paints are 70 generally composed of a mixture of gum (arabic gum) siccatives linseed oil and gasoline, in suitable proportions depending upon the paint having to be more or less fluid. Then to pour the previously molten and hot 75 protecting composition in a mould made of wood, metal, cardboard or other suitable material placed around the container and then to allow the said composition to freely set. To said coating is advantageously applied an 80 external layer of a watertight substance such as canvas or a rubber sheet and also an external gauze or wire mesh sheet or a similar 85 protecting sheathing.

For certain applications and particularly 90 when there is a risk of the container being hit by big gauge projectiles, a layer of a light and porous substance such as porous rubber, blotting paper or the like is advantageously provided between the container wall and the 95 resilient coating as thus the metal flange forced out by the passage of the bullet through the said wall will not damage the said coating but will merely tear open the 100 underlying layer of porous substance.

Owing to the resiliency of the protecting composition, if the container receives a hard 105 blow, it is protected as by a cushion whereas

if a bullet or projectile or a similar object passes through it, the perforation thereby produced is automatically and immediately closed up or sealed whereby any leakage of the fluid from the container is prevented with its concomitant disastrous risks when said fluid is of an inflammable nature such as gasoline. Such composition also possesses the great advantage that it can readily melt under the influence of heat and carbonize without being set on fire.

Thus it will be readily appreciated how useful the method according to the invention is, particularly for coating tanks used on board aeroplanes, hydroplanes, airships or like aircraft machines i. e. in all cases where any leakage of gasoline as a result of an accidental impact or perforation involves the risk of fire destroying the machine.

20 What I claim is:—

1. A method for protecting fluid containers and particularly tanks containing inflammable fluids as gasoline comprising the step of coating the container with a molten composition comprising suitable proportions of glycerine, a gelatine substance such as pure gelatine, fish glue, vegetable glue, arabic gum, and gum-lac, a binding substance such as glucose, molasses, treacle and water, somewhat similar to the composition used for covering printing rollers, and allowing said coating to set.

2. A method for protecting fluid containers particularly tanks containing inflammable fluids as gasoline comprising applying a thin layer of an adhesive paint to the outer wall of the container, encompassing said container with a corresponding mould of suitable material, pouring into said mould a previously molten and hot composition comprising glycerine, a gelatinous substance, a binding substance and water, allowing the composition to set, and removing the mould.

3. A method for protecting fluid containers particularly tanks containing inflammable fluids such as gasoline comprising applying a thin layer of an adhesive paint on the outer wall of the container, pouring into a mould encompassing said container a molten and hot composition comprising glycerine, a gelatinous substance, a binding substance and water, allowing the composition to set, removing the mould, and applying a layer of a substance adapted to form a protective sheathing.

4. A method for protecting fluid containers particularly tanks containing inflammable fluids as gasoline comprising applying on the outer wall of the container a

layer of a light and porous substance (such as porous rubber, blotting paper) then by means of a mould applying in the molten state a thicker layer of a composition comprising glycerine, a gelatinous substance, a binding substance and water, allowing the composition to set, removing the mould and applying a layer of a substance adapted to form a watertight and protective sheathing and comprising wire mesh.

5. A method for protecting fluid containers and particularly tanks containing inflammable fluids such as gasoline comprising the step of coating the container with a molten composition comprising in volume 30 to 50 parts of glycerine, 40 to 60 parts of a gelatinous substance, 1 to 2 parts of a binding substance and 10 to 15 parts of water, allowing said coating to set and applying a layer of a substance adapted to form a protective sheathing.

6. A method for protecting fluid containers and particularly tanks containing inflammable fluids as gasoline against impacts and perforations comprising the step of coating the container by means of a mould with a molten composition comprising in volume 39½ parts of glycerine, 48 parts of gelatine or fish glue, 1½ parts of commercial glucose or molasses and 11 parts of water, and allowing said coating to set.

7. A method for protecting fluid containers and particularly tanks containing inflammable fluids as gasoline comprising applying on the outer wall of the container a thin layer of an adhesive paint, pouring into a removable mould encompassing said container and made of a suitable material (such as wood, metal cardboard) a composition comprising 39½ parts of glycerine, 48 parts of gelatine or fish glue, 1½ parts of commercial glucose or molasses and 11 parts of water, allowing the composition to set, removing the mould and applying a layer of a substance adapted to form a watertight and protective sheathing and comprising wire mesh.

8. A fluid container provided on its outer wall with a composite coating produced according to the method as in claim 7.

9. A fluid container provided on its outer wall with "an adhering coating made of a composition comprising glycerine, a gelatinous substance such as gelatine or fish glue, a binding substance such as molasses or glucose and water, such a composition being similar to the one used for covering printing rollers."

In testimony whereof I affix my signature.

RENE COURTIN.